

June 27, 1967

J. V. WINKLER

3,328,067

SNOW SHOVEL

Filed Oct. 13, 1965



Fig. 1



Fig. 2

INVENTOR  
James V. Winkler

BY *John D. Meek*  
ATTORNEY

# United States Patent Office

3,328,067

Patented June 27, 1967

1

3,328,067

## SNOW SHOVEL

James V. Winkler, Midland, Mich., assignor to The Dow Chemical Company, Midland, Mich., a corporation of Delaware

Filed Oct. 13, 1965, Ser. No. 495,530  
1 Claim. (Cl. 294—54)

This invention relates to material handling devices and more particularly concerns an improved shovel for handling snow.

The object of the present invention is to provide as an article of manufacture a specially prepared shovel device, the blade of which is of treated magnesium base metal, having improved snow-handling qualities in that snow will not prematurely slip therefrom nor excessively adhere thereto whether being lifted or pushed.

Another object of the invention is to provide an improved snow shovel which permits easier handling of snow.

A further object of the invention is to provide an improved magnesium snow-handling device with improved corrosion and abrasion resistance.

The accompanying drawing illustrates one embodiment of the present novel shovel article of the invention as specially treated; which when considered in view of the following detailed description will serve to illustrate the invention, and wherein:

FIG. 1 is an isometric view of a "pusher" type shovel, having a curved blade treated in accordance with the present invention.

FIG. 2 is a partial cross-sectional view of the shovel blade of FIG. 1 showing the base metal and anodized coating.

The present novel shovel article comprises a snow shovel, equipped with an elongated handle which may either be of wood or metal or other suitable material, and a blade of anodized magnesium base metal. The anodizing of the magnesium or magnesium base alloy article (such as a shovel blade) usually is carried out by the process set forth in U.S. Patent 2,901,409. This is well known in the magnesium finishing art as the "Dow No. 17 process." In this process the blade is contacted with an aqueous solution at a temperature between 150° F. and the boiling point of the solution, at a voltage sufficient to produce sparking between the surface of the article and the solution. This aqueous anodizing solution consists of water in which is dissolved water-soluble inorganic compounds yielding the radicals ammonium, fluoride, phosphate, sodium, and hexavalent chromium in amount sufficient to produce in the solution an ammonium concentration between 3.2 and 15 percent, a fluoride concentration of at least 6 percent, a phosphorous concentration calculated as  $\text{PO}_4$  between 2 and 10 percent, a sodium concentration between 0.3 and 5.0 percent, and a hexavalent chromium concentration between 0.3 and 5.0 percent, and sufficient mineral acid to give the solution a pH of 0.5 to 4, the anodizing being continued for a time sufficient to give the surface of the article a tan or green color. Although the process taught in U.S. Patent 2,901,409 ordinarily is used in preparing the present novel article, it should be understood that other anodizing treatments for magnesium and magnesium alloys which provide an anodized surface hav-

2

ing substantially the same properties and characteristics as the Dow No. 17 process can be used.

The term "magnesium base metal" as used herein means the pure and commercial primary magnesium metal and magnesium base alloys in which the magnesium content is at least about 80 percent by weight.

Referring now to the drawing, there is shown a "pusher" type snow shovel comprising a long handle 10 rigidly but removably connected by a bracket 12 and bolt 14 to a curved magnesium base metal plate 16 having an anodized surface 18. If desired, of course, the surface of the blade not normally used to displace the snow need not be anodized.

The present novel material handling device is highly useful as a pusher or lifter type snow shovel in removing or displacing snow inasmuch as its anodized blade provides, highly desirable snow-holding and handling qualities (i.e., holding and releasing) by being sufficiently "sticky" or adherent to snow to prevent premature slippage of said snow therefrom but sufficiently non-adherent or "slippery" enough to avoid excessive sticking-on of the snow. In addition, the blade of the shovel so-anodized is corrosion and abrasion resistant.

The following example serves to illustrate the utility of the invention and the improved snow-handling qualities thereof:

### Example I

Actual use of six experimental shovels prepared in accordance with the present invention, all of the same shape, size and blade thickness, gave evidence of the superior qualities of these shovels in respect to the easy handling of snow while either pushing or lifting when compared to use of conventional shovels whose blade surfaces were of metallic aluminum, unanodized magnesium, painted or plastic coated metal. Most of the conventional shovels were so slippery that the snow load slid off prematurely at low angles to the horizontal, or so sticky that the snow load tended to cling too long to the shovel surface even at high angles to the horizontal. The anodized shovel blade in accordance with the present invention, however, reportedly exhibited just the right stickiness factor to provide unusually good snow control.

### Example II

In order to quantitatively, or at least more definitively, indicate the improvement in the snow-handling qualities of the present novel anodized shovel article, i.e., a desirable non-stickiness without either the stickiness or slippage associated with conventional snow shovel blades; various tests were performed as follows: a number of sheet metal channel sections were prepared to determine the angles of inclination to the horizontal at which snow would slide off or be retained on said sections. The snow-contacting surface included anodized magnesium, unanodized aluminum, unanodized magnesium, a conventionally painted magnesium surface, two magnesium surfaces with standard non-anodized chemical treatments, and anodized aluminum. The temperature during the tests was 36° F., and the relative humidity was 40 percent.

Though a very small amount of snow tended to stick to all the surfaces tested, the tests showed that the angles varied from, e.g., 10° to 90°, but that in every case the anodized magnesium varied midway between these ex-

tremes, with the average angle over several tests being about 33°. In actual tests with the present novel shovel, this blade angle proved to be very effective and desirable along with the general snow-handling properties of the anodized magnesium shovel. The shovel provided with the ski wax was extremely slippery, so much so that it was largely ineffective for use in handling snow. The painted AP10 shovel, on the other hand, in actual shovelling operations was found to be too sticky and its efficient use for handling snow was limited.

| Surface:                                                 | Approximate angle, deg. |
|----------------------------------------------------------|-------------------------|
| (1) Magnesium with Tedlar <sup>1</sup>                   | 10                      |
| (2) Aluminum—anodized                                    | 18                      |
| (3) Magnesium—bare                                       | 18                      |
| (4) Magnesium—ski wax                                    | 27                      |
| (5) Magnesium—anodized by Dow No. 17 treatment           | 33                      |
| (6) Magnesium—painted (Unichrome—AP10)                   | 36                      |
| (7) Magnesium(ferric nitrate <sup>2</sup> bright pickle) | 72                      |
| (8) Magnesium(chrome pickle) <sup>3</sup>                | 82                      |
| (9) Aluminum—bare                                        | 90                      |

<sup>1</sup> Trade name and particular paint composition designation of M & T Chemicals, Inc.

<sup>2</sup> Ferric nitrate bright pickle includes treatment in an aqueous solution comprising chromic acid, ferric nitrate, and potassium fluoride as described in bulletin entitled "Magnesium Finishing," page 69, published by The Dow Chemical Co., 1963.

<sup>3</sup> Chrome pickle includes treatment in an aqueous solution comprising sodium dichromate and nitric acid as described in bulletin entitled "Magnesium Finishing," page 53, published by The Dow Chemical Co., 1963.

These tests support and substantiate under controlled test conditions the marked improvement in snow-handling qualities of the anodized magnesium as used in shovels of the present invention in comparison to shovels of bare magnesium or aluminum, or with other of the commonly used finishes.

The present invention may be modified and changed without departing from the spirit or scope thereof, and it is understood that the invention is only limited as defined in the appended claim.

I claim:

An article of manufacture comprising a snow shovel having an elongated handle angularly connected to a magnesium base metal blade, at least the load carrying surface of said blade being anodized so as to retard and prevent premature slippage of shoveled snow carried thereon.

#### References Cited

#### UNITED STATES PATENTS

|           |         |        |        |
|-----------|---------|--------|--------|
| 127,405   | 6/1872  | Butler | 294—49 |
| 2,183,976 | 12/1939 | Smith  | 294—54 |

GERALD M. FORLENZA, Primary Examiner.

G. F. ABRAHAM, Assistant Examiner.